# EUROPEAN PATENT SPECIFICATION

(11) **EP 0 032 637 B1**
(45) Date of publication and mention of the grant of the patent: **22.05.1985**
(21) Application number: 80304771.1
(22) Date of filing: 31.12.1980
(51) Int. Cl.: D06M 13/40, D06M 13/26, D06M 15/564, D06M 15/693, D06M 15/248, D06M 11/00

(54) **Textile finishing**
Textilveredlung
Apprêt textile

(30) Priority: 16.01.1980 GB 8001470; 26.02.1980 GB 8006507
(43) Date of publication of application: 29.07.1981
(73) Proprietor: WOOL DEVELOPMENT INTERNATIONAL LIMITED, London, SW1Y 5AY (GB)
(72) Inventor: Benisek, Ladislav, Burley-in-Wharfedale West Yorkshire (GB); Craven, Penelope Christine, Saltair Shipley West Yorkshire (GB)
(74) Representative: Wharton, Peter Robert (GB)

## Description

This invention relates to a method of finishing keratinous fibres to render textile articles made from such fibres resistant to area felting shrinkage and flame-retardant.

Keratinous fibres, e.g. wool, are naturally flame retardant, but increasing stringency of regulations in various countries has meant that certain constructions of wool fabrics, or fabrics for certain end uses, e.g. in aeroplanes, and for clothing to provide protection against heat and flames, require an additional flame retardancy treatment. The titanium and zirconium flame retardancy treatments described in our U.K. Patent Nos. 1,372,694 and 1,379,752 have proved eminently suitable for improving the flame retardancy of wool textiles to meet the standards imposed by various legislative bodies.

The above treatments are fast to machine washing but, as is well-known, wool textiles tend, according to construction, to felt when washed in a machine and hence shrink. Many methods for rendering wool textiles shrink resistant are available but are in general not compatible with the above treatments because of curing difficulties at low pH values, or the shrink-resist polymer applied adds to the fuel contribution, i.e. increases the flammability, of the textile, thereby at least partly negating the flame retardancy treatment. Certain shrink-resist processes involving chlorination are not incompatible with the above treatments, nor do they add significantly to the fuel contribution of the textile, but are generally not desirable because chlorination lowers the water repellency and causes difficulties with dyestuffs. There is also the disadvantage of an extra processing step involving noxious chemicals.

According to the present invention there is provided a method of finishing keratinous textile articles which comprises treating the articles with an anti-felt polymer and an anionic titanium or zirconium complex characterised in that the anti-felt polymer is applied with a polymer of chlorinated ethylenically unsaturated monomer, and thereafter the articles are treated with the anionic titanium or zirconium complex at pH 4 or less.

The process is generally applicable to water-soluble curable shrink-resist polymers and prepolymers and especially those having ionic charges. Isocyanate functional polymers, and especially blocked isocyanate polymers, are preferred particularly water-soluble blocked isocyanates such as polycarbamoyl sulphonates. Examples of suitable polymers include polycarbamoyl sulphonates, Bunte salt polymers, the amphoteric polymers of our British Patent No. 1,547,958, and anionic acrylate emulsions. Cationic polymers such as a polyamideephichlorhydrin polymer, or azetidinium polymers, may also be used provided they are compatible with the chlorinated polymer emulsion used, if a cationic emulsion is employed. When the preferred chlorinated polymer emulsions are used, which are anionic, it is preferred to use anionic anti-felt polymers. Especially preferred are the polycarbamoyl sulphonates described in U.K. Patent No. 1,419,306. These may conveniently be prepared from polymeric di- or poly-isocyanates by treatment with sodium bisulphite.

Preferred polycarbamoyl sulphonates have polyoxyalkylene, e.g. polypropylene oxide, backbones and three carbamoyl sulphonate groups. Particularly preferred compounds have the following structure: wherein
n is about 13. Such a compound is available commercially under the name "Synthaprett BAP" trade mark of (Bayer).

Preferred curable polymeric materials have a polymeric chain backbone and at least two thiosulphate groups per molecule. The chain may advantageously be a polyoxyalkylene, e.g. polyoxypropylene, chain. Particularly preferred materials of this type have the following structural formula: where n is about 13.

Prepolymers of this type are disclosed in our British Patent No. 1,423,342. A suitable compound is available commercially under the trade mark "Lankrolan SHR3". It has been found that this type of polymer gives a very good handle to the treated fabric, especially when used with the "Neoprene" (trade mark) polymer mentioned hereinafter.

The polymer of a chlorinated ethylenically unsaturated monomer combines with the anti-felt polymer to give a shrink-resist effect, and thus allows less polymer to be used that would be necessary if it were used alone. Since the chlorinated polymers in general do not add to the fuel contribution of the textile and may even impart a degree of flame retardance, a net lowering of the fuel contribution of the shrink-resist treatment can be obtained. The surprising properties of these polymers lie in their capacity both to enhance the shrink-resist qualities of other polymers, particularly polycarbamoyl sulphonates and Bunte salts, and enhance the flame retardant properties of the titanium and zirconium complexes.

The chlorinated polymers which may be used include in general, polyvinyl chloride, polyvinylidene chloride, polychloroprene, and dichlorobutadiene. In general the higher the chlorine content of the polymer the better its flame retardancy characteristics, but this criterion is affected by other factors. Most of these polymers are too hard alone and therefore are available as copolymers with such monomers as acrylonitrile or methacrylic acid. The latter add to the fuel contribution of the copolymer and in certain cases may render the polymer unsuitable. In general most commercially available polyvinylchloride compositions are unsuitable.for this reason. We have found that for augmenting the shrink-resist effect (thereby allowing the use of less anti-felt polymer) while keeping the fuel contribution as low as possible, the preferred chlorinated polymers are Polidene 33-041 (a polyvinylidene chloride copolymer - trade mark of Scott Bader Co. Ltd.) and Neoprene 400 (a copolymer of polychloroprene and 2,3-dichloro-1,3-butadiene - Du Pont), especially the latter.

The treatment with titanium or zirconium may be carried as described in our above U.K. Patents. In brief the metals are applied, preferably by exhaustion as anionic complexes with flouride, citrato, or tartrato ions at a PH in the range 1 to 4. The titanium treatment is more effective, weight for weight, than the zirconium treatment but leads to a slight yellow colouration and should generally be used only with dark shades or where colouration is immaterial.

The quantities of agents may vary within wide limits subject to the desired degree of shrink-resistance, the flame retardancy required, and such factors as the substrate, coreactants, and so on. Thus in general the anti-felt prepolymer may be applied in the range 0.1 to 10% oww, preferably 0.2 to 2%, the lowest amount compatible with adequate shrink-resistance being chosen. The chlorinated polymer may be used in amounts of from 1 % to 10%, with 1. to 4% being preferred. The titanium or zirconium treatments may be applied in the ranges of 0.5% to 2.5% or 1% to 5% respectively (calculated as oxide) again depending on the substrate and the level of flame retardancy required.

The keratinous fibres may be for example mohair, alpaca, vicuna, angora, or especially wool, and the textile article may be in the form of loose stock, slivers, slubbings, rovings, yarns, fabrics, made-up garments or carpets, preferably fabrics.

The shrink-resist treatment may be carried out in any suitable manner e.g. exhaustion, dipping, spraying or padding, preferably the latter, and the flame retardancy treatment is preferably carried out by exhaustion from long liquor.

The invention will be illustrated further by the following examples. The test methods used were as follows

### Felting Shrinkage

This was determined after 1 hour and 3 hours in an International Cubex (trade mark) Washing Machine, using a phosphate buffer at PH7 and 40°C with liquor ratio 15:1, and total load 1 kg made up with polyester makeweights. The results are expressed as percentage area felting shrinkage.

### Flame-Resistance Test

This was evaluated according to Federal Aviation Regulations 25.853b, a vertical flame test with a 12 second ignition time. To meet this standard the after-burning time should not exceed 15 seconds and the char length should not be more than 20 cm (8 inches), tested in both the warp and weft directions. Wash fastness of the flame retardancy effect is determined after 10 and 20 washes in a Kenmore (trade mark) Model 21900 washing machine at 40°C, liquor ratio 1:36, load 1.8 kg using 90g "Bold" (trade mark) washing power per 65 litres.

### Examples 1 to 10

Lankrolan SHR3 and Neoprene 400 were padded onto a wool serge fabric. The fabric was dried and then cured at 150°C for 5 minutes. A titanium flame retardant treatment was applied by immersing the fabric at 1:20 liquor ratio in a bath containing 10% oww HCI (37%) 4% oww citric acid and 6% oww K₂TiF₆ for 30 minutes at 60°C, liquor ratio 1:30, by rinsing and drying.

The area felting shrinkage of the fabric after 3 hours test; and the FAR 25.853B test results are given in Table 1 below for a variety of component concentrations.

The Lankrolan SHR3 treatment is not compatible with the titanium flame-retardant treatments (Examples Nos. 1-3). The addition of Neoprene 400to the Lankrolan SHR3 not only makes the shrink-resist treatment compatible with the flame retardant treatment but it also allows a lower concentration of Lankrolan SHR3 to be used to achieve adequate shrink-resistance (Examples Nos. 4-10). In other words the incorporation of Neoprene 400 imparts flame-resistance to Lankrolan SHR3 and it also acts as a shrink-resist agent.

### Example 11

Synthappret BAP (0.4% oww) NaHC0₃ (1 % oww) and Neoprene 400 (3%) were padded onto a wool serge fabric. The fabric was dried and then cured at 140°C for 5 minutes. Zirconium flame retardant treatment was applied by immersing the fabric at 1:20 liquor ratio in a bath containing 10% oww HCI (37%), 4% oww citric acid and 8% oww K₂ZrF₆ for 30 minutes at 70°C, followed by rinsing and drying.

The area felting shrinkage of the fabric was zero after 1 hour and 2% after 3 hours test; and the fabric passed the FAR 25.853b test in both the warp and weft directions. It was also observed that the smooth drying properties of the fabric given this treatment was exceptionally good, and that the spray rating, according to B.S. 3702, was unchanged by the treatment. A similar fabric given a chlorination treatment showed a marked deterioration in spray rating.

### Examples 12 to 19

In these examples the Synthappret and Polidene were applied to various fabrics by a pad-dry-cure route and the "Zirpro" zirconium flame retardant treatment was applied as in Example 11. The results are given in the Table 2 below.

### Example 20

An all-wool gaberdine fabric, 270 g/m², was treated with 1.25% Synthappret BAP, 1.25% Neoprene 400 and 1 % NaHC0₃ by the pad-dry-cure technique, curing being achieved by heating to 150°C for 5 minutes. Thereafter, in a separate bath, the fabric was given a Zirpro treatment with 10% Hêl (37%), 4% citric acid, and 6% K₂ Ti F₆ for 30 minutes at 70°C at a fabric-to-liquor ratio of 1:25.

The results are given in Table 3 below.

### Example 21

Example 20 was repeated with the inclusion of 3% FC214 (a fluorocarbon supplied by the 3M Company) in the Zirpro treatment.

As can be seen from Table 3 below, this resulted in a fabric which was shrink-resistant, flame retardant, and oil-and water-repellant, the first three properties being fast to severe washing at 60°C and the last fast to at least 20 washes at 40°C.

Thus it can be seen that the process of the invention enables a shrink-resistant and flame retardant finish to be applied to wool fabrics by a simple route using commercially available chemicals, without adversely affecting properties such as water-repellency.

## Claims

1. A method of finishing keratinous textile articles which comprises treating the articles with an anti-felt polymer and an anionic titanium or zirconium complex characterised in that the anti-felt polymer is applied with a polymer of a chlorinated ethylenically unsaturated monomer, and thereafter the articles are treated with the anionic titanium or zirconium complex at pH 4 or less.

2. A method according to claim 1 in which the anti-felt polymer is an isocyanate functional polymer or a Bunte salt functional polymer.

3. A.method according to claim 2 in which the polymer is a polycarbamoyl sulphonate.

4. A method as claimed in claim 2 in which the polymer has the following structure: OR wherein n is about 13.

5. A method as claimed in any one of claims 1 to 4 in which the chlorinated polymer is polyvinylchloride, polyvinylidene chloride, polychloroprene, or dichlorobutadiene.

6. A method as claimed in claim 5 in which the chlorinated polymer is a copolymer of polychloroprene and 2,3-dichloro-1,3-butadiene.

7. A method according to any one of claims 1 to 6 in which the titanium or zirconium is applied by exhaustion as an anionic complex with flouride, citrato, or tartrato ions at a pH in the range of 1 to 4.

8. A method according to any one of claims 1 to 7 in which the anti-felt polymer is present on the articles in the range 0.2 to 2% by weight the chlorinated polymer is present on the articles in the range 1 to 4% by weight and the titanium or zirconium is present in the range 0.5 to 2.5% or 1% to 5% by weight respectively (calculated as oxide).

9. A method as claimed in any one of claims 1 to 8 in which the keratinous fibres are wool fibres.

10. A method as claimed in any one of claims 1 to 9 in which the textile article is a fabric.

11. A method as claimed in any one of claims 1 to 10 in which the polymers are applied by exhaustion, dipping, spraying or padding.

## Revendications

1. Procédé pour l'apprêtage d'articles textiles kératiniques qui consiste à traiter les articles avec un polymère anti-feutrage et un complexe anionique titane ou zirconium, caractérisé en ce qu'on applique le polymère anti-feutrage avec un polymère d'un monomère chloré éthyléniquement non saturé, après quoi, on traite les articles avec le complexe anionique titane ou zirconium à un pH de 4 ou moins.

2. Procédé selon la revendication 1, caractérisé en ce que le polymère anti-feutrage est un polymère fonctionnel d'isocyanate ou un polymère fonctionnel d'un sel de Bunte.

3. Procédé selon la revendication 2, caractérisé en ce que le polymère est un sulfonate de polycarbamoyle.

4. Procédé selon la revendication 2, caractérisé en ce que le polymère présente la structure suivante: ou où n est égal à environ 13.

5. Procédé selon l'une quelconque des revendications 1 à 4, caractérisé en ce que le polymère chloré est du chlorure de polyvinyle, de polyvinylidène, du polychloroprène ou du dichlorobutadiène.

6. Procédé selon la revendication 5, caractérisé en ce que le polymère chloré est un copolymère de polychloroprène et de 2,3-_{d}ichloro-1,3-butadiène.

7. Procédé selon l'une quelconque des revendications 1 à 6, caractérisé en ce que le titane ou le zirconium est appliqué par épuisement sous forme de complexe anionique avec des ions de fluorure, citrate ou tartrate, à un pH de l'ordre de 1 à 4.

8. Procédé selon l'une quelconque des revendications 1 à 7, caractérisé en ce que le polymère anti-feutrage est présent sur les articles à raison de 0,2 à 2% en poids, le polymère chloré est présent sur les articles à raison de 1 à 4% en poids et le titane ou le zirconium est présent à raison de 0,5 à 2,5% ou de 1 à 5% en poids, respectivement (calculé sous forme d'oxyde).

9. Procédé selon l'une quelconque des revendications 1 à 8, caractérisé en ce que les fibres kératiniques sont des fibres de laine.

10. Procédé selon l'une quelconque des revendications 1 à 9, caractérisé en ce que l'article textile est un tissu.

11. Procédé selon l'une quelconque des revendications 1 à 10, caractérisé en ce que les polymères sont appliqués par épuisement, trempage, aspersion ou tamponnage.

## Patentansprüche

1. Verfahren zum Appretieren von keratinhaltigen Textilartikeln, das umfaßt das Behandeln der Artikel mit einem Antifilz-Polymeren und einem anionischen Titan- oder Zirkonium-Komplex, dadurch gekennzeichnet, daß das Antifilz-Polymere aufgebracht wird zusammen mit einem Polymeren eines chlorierten, ethylenisch ungesättigten Monomeren und daß danach die Artikel mit dem anionischen Titan-oder Zirkonium-Komplex bei pH 4 oder weniger behandelt werden.

2. Verfahren nach Anspruch 1, worin das Antifilz-Polymere ein Isocyanat-funktionelles Polymeres oder ein Bunte-Salz-funktionelles Polymeres ist.

3. Verfahren nach Anspruch 2, worin das Polymere ein Polycarbamoylsulfonat ist.

4. Verfahren nach Anspruch 2, worin das Polymere die folgende Struktur hat: oder worin n etwa 13 bedeutet.

5. Verfahren nach einem der Ansprüche 1 bis 4, worin das chlorierte Polymere Polyvinylchlorid, Polyvinylidenchlorid, Polychloropren oder Dichlorobutadien ist.

6. Verfahren nach Anspruch 5, worin das chlorierte Polymere ein Copolymeres von Polychloropren und 2,3-Dichloro-1,3-butadien ist.

7. Verfahren nach einem der Ansprüche 1 bis 6, worin das Titan oder Zirkonium aufgebracht wird durch Ausschöpfen in Form eines anionischen Komplexes mit Fluorid-, Citrat- oder Tartrationen bei einem pH-Wert innerhalb des Bereiches von 1 bis 4.

8. Verfahren nach einem der Ansprüche 1 bis 7, worin das Antifilz-Polymere auf den Artikeln vorliegt in einer Menge innerhalb des Bereiches von 0,2 bis 2 Gew.-%, das chlorierte Polymere auf den Artikeln vorliegt in einer Menge innerhalb des Bereiches von 1 bis 4 Gew.-% und daß Titan oder Zirkonium vorliegt in einer Menge innerhalb des Bereiches von 0,5 bis 2,5 Gew.-% bzw. 1 bis 5 Gew.-% (berechnet als Oxid.).

9. Verfahren nach einem der Ansprüche 1 bis 8, worin die keratinhaltigen Fasern Wollfasern sind.

10. Verfahren nach einem der Ansprüche 1 bis 9, worin der Textilartikel ein Gewebe ist.

11. Verfahren nach einem der Ansprüche 1 bis 10, worin die Polymeren durch Ausschöpfen, Eintauchen, Aufsprühen oder Aufklotzen aufgebracht werden.
